

# UNITED STATES PATENT OFFICE.

SAMUEL PEACOCK, OF WHEELING, WEST VIRGINIA, ASSIGNOR, BY MESNE ASSIGNMENTS, TO WHEELING STEEL & IRON COMPANY, OF WHEELING, WEST VIRGINIA, A CORPORATION OF WEST VIRGINIA.

## PROCESS OF COATING STEEL SHEETS WITH TIN.

1,396,051.

Specification of Letters Patent.

Patented Nov. 8, 1921.

No Drawing.

Application filed November 9, 1920. Serial No. 422,813.

To all whom it may concern:

Be it known that I, SAMUEL PEACOCK, a citizen of the United States, residing at Wheeling, in the county of Ohio and State 5 of West Virginia, have invented certain new and useful Improvements in Processes of Coating Steel Sheets with Tin; and I do hereby declare the following to be a full, clear, and exact description of the invention, such as will enable others skilled in 10 the art to which it appertains to make and use the same.

This invention relates to a process of 15 coating thin steel sheets with tin, and has for its object to improve the procedures heretofore proposed.

With these and other objects in view, the 20 invention consists in the novel steps and combinations of steps constituting the process, all as will be more fully hereinafter disclosed and particularly pointed out in the claims.

In order that this invention may be the 25 more clearly understood, it is said: In the present procedure of coating one metal with another, such, for example, as coating thin sheets of mild steel with tin, to form the "tin plate" of commerce, it is usual to free the steel sheets of oxids, grease, etc., and to 30 then immerse them in a molten bath containing tin, at atmospheric pressure.

The differences in contraction between 35 the steel plates and the tin coatings on cooling, although very small, are, yet, sufficient to form fissures or cracks in the very thin tin coatings now employed.

These fissures are usually too small to be 40 readily detected by magnifying glasses, but may be readily detected by well known chemical tests, and they offer a sufficient exposure of the steel through the tin coating to start an electrolytic action when immersed in an electrolytic solution, such, for example, as is afforded by many food products, 45 such as fruits and vegetables, when put up in tin cans.

It therefore follows that for many industrial uses the present tin plates have a 50 short life due to the inevitable corrosion that follows their use, and the very serious, well known objections that said corrosion entails in producing salts that may be injurious to health.

It has been attempted to avoid these objec-

tions by depositing the tin coating electrolytically on the steel plate, but such coatings invariably have a crystalline structure, and are found in practice to be as objectionable from a sanitary point of view as is a coating produced from a molten bath. That is to say, it has proved in practice that when electrolytically deposited coatings of tin have been employed on cans containing fruits and vegetables, an electric circuit is formed between the tin and steel about as often as is the case when said coatings are provided from a molten bath, and therefore, no progress toward a solution of the difficulty is made.

I have discovered, on the other hand, that if instead of immersing the thin steel sheets in a coating bath of molten tin, under substantially atmospheric pressure, I substitute a solution of a tin salt, such as stannous chlorid  $\text{SnCl}_2$ , and if I increase the pressure by means of heat to from say 5 to 15 atmospheres or higher, the advantages described below are attained. That is to say, I have discovered if I maintain a low ionic concentration in the tin salt solution, it will deposit out the tin in a colloidal state, instead of in a crystalline state, and the steel will be covered completely and without fissures with said tin.

On the other hand, a low ionic concentration means a slow rate of coating. But I have observed that by heating the coating solution while maintaining a super-atmospheric pressure, thereon, the rate of deposition is increased. This is especially true, if the solution is agitated and the pressure is maintained at a point sufficient to prevent boiling of the coating solution. This may be readily accomplished by the use of an autoclave.

I have further observed that the degree of 95 ionic concentration governs the colloidal nature of the metal coating, or the lower the ionic concentration, the more colloidal will be the deposited tin. But care must be taken to not employ such a low ionic concentration as will render the rate of coating so slow as to be commercially inoperative.

As a practical operation in carrying out 100 this invention, I may use, say, 5 parts by weight of the stannous chlorid to 100 parts by weight of the diluent to be used, such as an ammonium alum or an alkali bi-tartrate.

I may next make up a 3% solution of said chlorid and alum or bitartrate with water. This said solution together with the sheets to be coated are placed in an autoclave under 5 a steam pressure of say between 5 and 15 atmospheres, or preferably of about 10 atmospheres, when the tin will be found to be coated on the steel sheets in a firmly adhering non-porous, non-fissured condition, much 10 superior to the coatings of the prior processes.

The plates are next removed from the autoclave, and dried, when they are ready for use in making tin cans, or other articles.

15 The function of the ammonium alum or the potassium or sodium bitartrate is to lower or restrain the natural ionic concentration of the stannous chlorid. But, of course, other restrainers may be employed. 20 The function of the heat is undoubtedly to increase the kinetic energy of the tin ions. Of course, the plates or sheets should be in a clean condition, or free from scale, grease, etc., before being immersed in the solution. 25 The latter should not have a concentration as high as 20% of the stannous chlorid, and from 3% to 5% is preferable.

It is obvious that those skilled in the art may vary the details of the procedure without departing from the spirit of the invention, and therefore, I do not wish to be limited to the above disclosure except as 30 may be required by the claims.

What I claim is:

85 1. The process of forming a coherent coating of tin on thin steel sheets which consists in preparing a solution of stannous chlorid mixed with an alum having an alkaline reaction adapted to restrain the ionic 40 concentration of said stannous chlorid; immersing said sheets in a clean condition in

said solution; and subjecting the latter to a steam pressure exceeding two atmospheres, substantially as described.

2. The process of forming a coherent 45 coating of tin on thin steel sheets which consists in preparing a solution of stannous chlorid mixed with an alkali alum salt adapted to restrain the ionic concentration of said stannous chlorid; immersing said 50 sheets in a clean condition in said solution; and subjecting the latter to a steam pressure exceeding five atmospheres, substantially as described.

3. The process of forming a coherent coating 55 of tin on thin steel sheets which consists in preparing a solution of stannous chlorid mixed with an ammonium alum adapted to restrain the ionic concentration of said stannous chlorid; immersing said 60 sheets in a clean condition in said solution, and subjecting the latter to a steam pressure exceeding five atmospheres, substantially as described.

4. The process of coating thin steel sheets 65 with tin which consists in preparing a solution containing stannous chlorid, and an ammonium alum; immersing said sheets in a clean condition in said solution; and subjecting said solution to a steam pressure 70 exceeding five atmospheres, substantially as described.

5. The process of coating thin steel sheets with tin which consists in preparing a solution containing less than 20% of stannous 75 chlorid and ammonium alum; immersing said sheets in a clean condition in said solution; and subjecting said solution to a steam pressure exceeding five atmospheres, substantially as described.

In testimony whereof I affix my signature.  
SAMUEL PEACOCK.